

Dec. 4, 1956

H. J. DAILEY

2,772,861

RADIATOR FOR ELECTRON DISCHARGE DEVICE

Original Filed June 29, 1951

Fig. 1.



Fig. 2.



Fig. 3.



INVENTOR

H. J. DAILEY

BY *J. Kelly*

ATTORNEY

# United States Patent Office

2,772,861

Patented Dec. 4, 1956

1  
2,772,861

## RADIATOR FOR ELECTRON DISCHARGE DEVICE

Hampton J. Dailey, deceased, late of Verona, N. J., by  
Ruth M. Dailey, executrix, Verona, N. J., assignor to  
Westinghouse Electric Corporation, East Pittsburgh,  
Pa., a corporation of Pennsylvania

Original application June 29, 1951, Serial No. 234,216.  
Divided and this application September 28, 1953, Serial  
No. 382,538

### 2 Claims. (Cl. 257—263)

This invention is a division of application S. N. 18  
234,216, filed June 29, 1951, now abandoned, and relates  
to radiators and more particularly, to radiators for elec-  
tron discharge devices.

Present day transmitting tubes included in the general  
classification of electron discharge devices, are the source  
of intense heat during operation, and require radiators  
of good thermal conductivity and adequate surface area  
to disperse the generated heat. Radiators employing  
copper fins have been commonly used. While the tubes  
alone are relatively light, not usually exceeding twenty-  
five pounds, the copper radiators may be several hundred  
pounds, and thus require a crew of several men or a crane  
to handle and to make tube replacements as needed from  
time to time. If it were possible to merely substitute  
aluminum or other light-weight metal or alloy for the  
copper in fabrication of the radiators, great saving of  
weight would be accomplished as density of aluminum is  
approximately 168 pounds per cubic foot as compared  
with 555 pounds for copper. However, until now, the  
fabrication of a radiator of aluminum, magnesium or  
alloy thereof and assembly with a transmitting tube has  
been found to have substantial limitations. A prerequi-  
site for a successful radiator is that it must have a secure  
bond with the copper anode of the transmitting tube, but  
aluminum, for example, when fabricated, quickly forms  
a very stable oxide surface to which it is, for all prac-  
tical purposes, impossible to make a good solder joint.  
This lack of adequate bond with the anode has prevented  
adoption of aluminum radiators for transmitting tubes,  
and similarly has prevented adoption of radiators of other  
light-weight metals and alloys.

Accordingly, the fundamental purpose of the present  
invention, is to provide a practical radiator of light-  
weight material, such as aluminum, for an electron dis-  
charge device and particularly for a transmitting tube  
in that classification.

Also, in general terms, an object of the invention is  
to provide an improved radiator of light-weight material  
such as aluminum adaptable to attachment to a copper  
anode of an electron discharge device with a secure bond  
therewith.

More specifically, an object of the invention is to in-  
clude within the radiator a means by which secure at-  
tachment between radiator and anode may be obtained.

Another object of the invention is to provide a liner  
for the radiator which can be soldered to the anode.

Yet another object of the invention is to obtain a  
complete bond between the liner and the radiator hub  
or body.

A further object of the invention is to provide an im-  
proved method of fabrication.

Still other objects of the invention will appear to those  
skilled in the art to which it appertains as the description  
proceeds, both by direct recitation thereof and by im-  
plication from the context.

Referring to the accompanying drawings, in which like

2

numerals of reference indicate similar parts throughout  
the several views:

Fig. 1 is a longitudinal section of a radiator fabricated  
in accordance with the present invention and shown ap-  
plied to an anode, which is depicted partly in section  
and partly in elevation;

Fig. 2 is a transverse section on line II—II of Fig. 1; and

Fig. 3 is a mid-sectional view of the central hub of  
the radiator shown in Figs. 1 and 2 at one step in the  
course of its fabrication.

In the specific embodiment of the invention illustrated  
in said drawings, the reference numeral 10 designates an  
electron discharge device in general, having usual triode  
or other electrodes of which the anode 11 shown herein  
is formed as part of the envelope with which it is appro-  
priately sealed so as to be evacuated, the lower end of  
said anode being closed as by an integrally formed dome  
12. The anode is usually made of copper and in the con-  
struction shown is an exterior part of the tube so as to  
be available for heat dissipation.

The radiator, designated in general by numeral 13,  
comprises a hollow body or hub 14 from which, in  
radial planes, project a plurality of fins 15. The pres-  
ent invention contemplates use of light-weight metal, such  
as aluminum, magnesium or alloys thereof, as the mate-  
rial of which said hub 14 and fins 15 are fabricated.  
The exterior cylindrical surface of the hub is milled with  
a plurality of longitudinal grooves 16, one for each fin,  
and the inner edges of the fins are applied in the grooves  
and brazed or otherwise securely attached throughout  
their engaging portions with the hub.

The interior of the radiator body or hub is provided  
with means for enabling the body to be securely attached  
to the anode throughout the juxtaposed surfaces after  
telescoping the said body upon the anode. According to  
the present invention, a metallic liner 17 is made integral  
with the said hub and constitutes the inner surface of the  
radiator body. Said liner is integrated with the hub so  
as to transmit heat by conduction from the anode to the  
hub and fins, and is of copper like the anode. The lower  
end of the liner 17 is hollowed to substantially conform  
to the curvature of dome 12.

In carrying out the method of fabrication, the liner  
is submerged to a point just below its rim in a pot of  
molten aluminum 21 or equivalent metal, kept in its  
fluid state by inclusion in an electrically heated pot 22.  
In view of the direct contact of the outer surface of the  
liner with the molten aluminum, an excellent bond will  
form at the outer surface of the liner 17 because copper  
is soluble in molten aluminum. The liner may be kept  
cooler than the surrounding aluminum by any appropriate  
means (for instance insertion inside it of a massive slug of  
cooled copper) whereupon a shell of solidified aluminum  
will form, growing radially outward from the liner 17.  
When the desired wall-thickness of solidified aluminum  
has formed, the unit may be withdrawn from the molten  
bath; or alternatively the heat may be shut off from the  
molten aluminum when the liner 17 is first immersed in  
it, and the whole mass of the molten aluminum be allowed  
to solidify. Solidification from the core radially out-  
ward insures against the formation of pores and blow-  
holes in the casting.

When the unit thus formed has cooled, it is machined  
to the desired size, and suitable slots to engage the inner  
edges of the fins are milled on its exterior surface. The  
fins may then be brazed into position.

After cleaning, solder is then introduced into the hol-  
low of the radiator and heat applied until the solder is  
liquefied, flux is added, and the anode is then pressed  
into the hollow of the radiator until solder extrudes at

the top of the radiator cavity and the parts have desired relation. The solder will harden and tenaciously adhere to the liner and to the anode and provides an excellent heat-conductive path from the anode to the radiator. The solder performs the function of providing a secure bond which will not deteriorate by oxidation.

By providing a structure enabling the radiator to be fabricated from aluminum or equivalent metal, a relatively light-weight radiator is obtained, and as comparative weights, it may be pointed out that where a prior art copper radiator weighed 225 pounds, an equivalent aluminum radiator in accordance with the present invention weighs only 98 pounds, thereby enabling one man to make a tube replacement in service. Since handling can be done by one man, the apparatus may be more compactly arranged, thus saving space in the transmitter station. Furthermore, providing lighter weight radiators of the present invention reduces shipping costs considerably.

**I claim:**

1. A electron discharge device comprising a copper anode, an aluminum radiator mounted on said anode, a liner of copper interposed between the anode and radiator, with a fused copper-aluminum bond integrating said liner and radiator as a unit, and solder interposed between said anode and liner securing the said liner on the anode.
2. A hollow radiator for an electron discharge device comprising an aluminum hub, fins projecting from said hub, a liner of copper within said hub and providing an inner surface for the hollow of the radiator to which solder will adhere, and a coating of copper-aluminum alloy interposed between and adherent to both the liner and the hub inseparably integrating the liner and hub as a unit.

1. An electron discharge device comprising a copper anode, an aluminum radiator mounted on said anode, a liner of copper interposed between the anode and radiator, with a fused copper-aluminum bond integrating said liner and radiator as a unit, and solder interposed between said anode and liner securing the said liner on the anode.

2. A hollow radiator for an electron discharge device comprising an aluminum hub, fins projecting from said hub, a liner of copper within said hub and providing an inner surface for the hollow of the radiator to which solder will adhere, and a coating of copper-aluminum alloy interposed between and adherent to both the liner and the hub inseparably integrating the liner and hub as a unit.

References Cited in the file of this patent

UNITED STATES PATENTS

- 2,181,366 Edwards et al. \_\_\_\_\_ Nov. 28, 1939  
20 2,288,380 Wing \_\_\_\_\_ June 30, 1942